

# United States Patent Office

3,127,347

Patented Mar. 31, 1964

1

3,127,347

## LUBRICATING COMPOSITION

Raymond A. Franz, El Dorado, Ark., assignor to Monsanto Chemical Company, St. Louis, Mo., a corporation of Delaware  
No Drawing. Filed May 20, 1960, Ser. No. 30,431  
4 Claims. (Cl. 252—28)

The present invention relates to a lubricating composition. More particularly, this invention relates to the use of tetraalkyl ureas as lubricating compounds.

The lubricating properties of nitrogen containing compounds have been rather extensively investigated. As a result many of these compounds have been found to exhibit excellent lubricating properties while others have shown very poor results.

It is then an object of this invention to provide a new and improved lubricating composition. It is another object of this invention to provide a new and improved lubricating composition comprised of particular nitrogen containing compounds. A more specific object of this invention is to provide a new and improved lubricating oil comprised of a tetraalkyl urea. Another specific object of this invention is to provide a new and improved lubricating grease comprised of a tetraalkyl urea and a minor amount of a thickening agent. Still another object of this invention is to provide a new and improved lubricating composition comprised of a tetraalkyl urea and a conventional petroleum lubricating composition. Additional objects will become apparent from the description of the invention.

In fulfillment of these objects, it has been found that tetraalkyl ureas possess very good lubricating properties and are especially adapted to utility as high temperature lubricants. The tetraalkyl ureas of this invention are represented by the formula:



wherein R<sub>1</sub>, R<sub>2</sub>, R<sub>3</sub>, and R<sub>4</sub> represent alkyl radicals each containing at least two carbon atoms, but not more than 18 carbon atoms. These ureas can be used per se as high temperature lubricants and also as the fluid base for high temperature greases. The tetraalkyl lubricants of this invention are useful at temperatures ranging from —62° to 325° C. and higher.

To facilitate understanding of the invention herein disclosed, the following examples are presented. It is to be understood, of course, that these examples are in no way to be construed as limiting the application, conditions, or operations of this invention.

### EXAMPLE I

A sample of 1,1-di-n-dodecyl-3,3-di-2-ethyl hexyl urea was subjected to a standard Four Ball Wear Test. The test was carried out at 1250 r.p.m. for two hours, steel on steel. The results were as follows:

| Temperature | Scar Diameters   |                  |
|-------------|------------------|------------------|
|             | 10 kg. load, mm. | 40 kg. load, mm. |
| 167° F.     | 0.37             | 0.51             |
| 400° F.     | 0.56             |                  |

These low scar diameters indicate good lubricating characteristics, superior to mineral oil and the more conventional high temperature hydraulic fluids.

2

### EXAMPLE II

The following additional test was used for determining the lubricating qualities of tetra-substituted ureas:

5 A 5/8 inch spindle with a polished, stainless steel head was placed in the socket of a drill press which was set at 1000 r.p.m. Enough of the indicated urea was placed in a 1 oz. tin to sufficiently cover the bottom of the tin. The rotating spindle was lowered into the tin and held in position with a nine-pound weight attached to the horizontal bar of the drill press. The spindle was allowed to run in this position for two minutes, after which time it was raised and the results of the test observed. After each test the spindle was polished with No. 3 emery cloth. The criterion for judging the lubricating qualities of the ureas is a comparison with a General Electric silicone oil, No. 81406. The results of this testing of several representative tetraalkyl ureas are given in the following table.

| Lubricating composition:                  | Lubricating quality |
|-------------------------------------------|---------------------|
| 1,1-di-n-octyl-3,3-di-n-octadecyl urea    | Good                |
| 1,1-di-n-hexyl-3,3-di-n-octadecyl urea    | Good                |
| 1,1-di-n-butyl-3,3-di-n-octadecyl urea    | Good                |
| 1,1-di-n-dodecyl-3,3-di-n-octyl urea      | Fair                |
| 1,1-di-n-dodecyl-3,3-di-2-ethylhexyl urea | Fair                |
| 1,1,3,3-tetra-n-octyl urea                | Fair                |
| G.E. silicone oil                         | Poor                |

### EXAMPLE III

30 Since thermal stability is necessary for high temperature lubricants, the following test was used to determine the amount of decomposition of several representative tetraalkyl ureas.

35 One gram of tetraalkyl urea was placed in a 10 x 75 mm. test tube which was immersed in a metal (Wood's alloy) bath. The temperature of the bath was raised to 200° C. and maintained for 20 minutes, after which time the temperature was raised to 250° C. for 20 minutes, and then to 300° C. for 20 minutes. At five minute intervals 40 the tubes were checked for discoloration and decomposition. At such intervals the vapors from the sample were tested for free amine with ammonia test paper dipped in ethanol.

45 The results of the testing of several representative tetraalkyl ureas is given in the following table:

| Lubricating Composition                   | Visible Decomposition | Amine Test /° C. |
|-------------------------------------------|-----------------------|------------------|
| 1,1-di-n-octyl-3,3-di-n-octadecyl urea    | Negative              | Negative         |
| 1,1-di-n-hexyl-3,3-di-n-octadecyl urea    | do                    | Do               |
| 1,1-di-n-butyl-3,3-di-n-octadecyl urea    | do                    | Do               |
| 1,1-di-n-dodecyl-3,3-di-n-octyl urea      | do                    | Do               |
| 1,1-di-n-dodecyl-3,3-di-2-ethylhexyl urea | do                    | Do               |
| 1,1,3,3-tetra-n-octyl urea                | do                    | Slight/300°      |

### EXAMPLE IV

60 A grease was prepared from 1,1-di-n-dodecyl-3,3-di-n-octyl urea by thickening with 15% by weight of finely divided (less than 1 micron particle size) SiO<sub>2</sub>. A 1 gram sample of this was then placed in a bicycle bearing. The conditions of the test were 430° F. and 1800 r.p.m. The grease showed low loss, good coating characteristics and no separation.

### EXAMPLE V

65 A grease was prepared from 1,1-di-n-hexyl-3,3-di-n-octadecyl urea by thickening with 15% by weight of finely divided (less than 1 micron particle size) SiO<sub>2</sub>. A 1 gram sample of this was then placed in a bicycle bearing. The conditions of the test were 430° F. and 1800 r.p.m. The grease showed low loss, good coating characteristics and no separation.

To further exemplify the utility of the tetraalkyl ureas as lubricating oils, Table I lists the viscosity index and pour point for a number of representative tetraalkyl ureas.

Table I

| Compound                                        | Viscosity Index | Pour Point, ° F. |
|-------------------------------------------------|-----------------|------------------|
| 1,1,3,3 tetra ethyl urea-----                   | 54              | -81              |
| 1,1 di-ethyl 3,3 di-2, ethyl hexyl urea-----    | 80              | -80              |
| 1,1,di-n-butyl 3,3, di-n-octyl urea-----        | 68.1            | -81              |
| 1,1,3,3 tetra n-hexyl urea-----                 | 68              | -69              |
| 1,1-di-n-hexyl 3,3-di-n-octyl urea-----         | 110             | -20              |
| 1,1-di-n-butyl 3,3-di-n-dodecyl urea-----       | 129             | -30              |
| 1,1-ki-2-ethyl hexyl 3,3-di-n-octyl urea-----   | 91.6            | -59              |
| 1,1,3,3-tetra-n-octyl urea-----                 | 127.5           | +5               |
| 1,1-di-n-dodecyl 3,3-di-n-hexyl urea-----       | 136             | -40              |
| 1,1-di-n-dodecyl 3,3-di-2-ethyl hexyl urea----- | 110.1           | -28              |
| 1,1-di-n-dodecyl 3,3-di-n-octyl urea-----       | 137.41          | +14              |
| 1,1-di-n-butyl 3,3-di-n-octadecyl urea-----     | 139             | +40              |
| 1,1-di-n-hexyl 3,3-di-n-octadecyl urea-----     | 136             | +25              |
| 1,1-di-n-octyl 3,3-di-n-octadecyl urea-----     | 138.4           | +35              |

The tetraalkyl urea lubricating compounds of this invention may be prepared by reacting a dialkyl carbamyl chloride having the formula



with a dialkylamine having the formula



wherein R<sub>1</sub>, R<sub>2</sub>, R<sub>3</sub>, and R<sub>4</sub> represent alkyl radicals each containing at least two carbon atoms preferably at an elevated temperature and in an inert diluent on reaction medium. The procedure for preparing the novel ureas of this invention can be varied substantially. While equimolecular proportions of the reactants are advantageously used, excessive quantities of either can be used if desired as dictated by economic or yield considerations. While it is not necessary to do so, the reaction is best carried out in the presence of an HCl-acceptor. Any alkaline agent which does not react to any serious degree with either of the reactants can be used. Tertiary alkylamines are particularly useful.

The reaction is preferably, but not necessarily, carried out in an inert diluent or reaction medium. Aliphatic and aromatic hydrocarbons are particularly useful in this regard.

The temperature of the reaction can be varied substantially. Elevated temperatures in the range of from about 50° C. to 200° C. are preferred.

When it is desired to use the tetraalkyl urea lubricants disclosed herein as lubricating greases, any conventional thickening agent may be used. Several non-limiting examples of such thickening agents are  $\text{SiO}_2$ , calcium base soap, sodium base soaps, etc. As illustrative of the use

of soap thickening agent, with the tetraalkyl lubricants at 235° F. a sodium base grease made with 1,1-di-n-octyl-3,3-di-n-octadecyl urea performed just as well as a sodium base grease made from a commercial lube oil.

5 The amount of thickening agent will be dependent upon the agent employed and the thickness desired for the grease. In the practice of the present invention, no thickening agent is necessary, although if used, an amount of thickening agent of from 5 to 20% by weight is preferred, although more or less may be used.

The lubricants of this invention may find utility in a host of applications. Several non-limiting examples of applications are lubricating oils, lubricating greases, hydraulic fluids or in any other utility requiring compounds having the physical characteristics set forth in the examples.

The lubricating compositions of this invention can be used in admixture with petroleum lubricating oils and greases. These tetraalkyl ureas may be present in such mixture in quantities ranging from 1 to 100 percent by weight. By addition of tetraalkyl lubricants to petroleum lubricants, certain properties of the petroleum lubricants may be improved.

What is claimed is:

25 1. A lubricating grease consisting essentially of a major amount of a tetraalkyl urea having the formula



wherein  $R_1$ ,  $R_2$ ,  $R_3$  and  $R_4$  represent alkyl radicals containing at least 2 carbon atoms and not more than 18 carbon atoms, thickened to grease-like consistency with a minor amount of a thickening agent.

2. A lubricating grease as described in claim 1 wherein the urea is 1,1-di-n-dodecyl-3,3-di-n-octyl urea.

3. A lubricating grease as described in claim 1 wherein the urea is 1,1-di-n-hexyl-3,3-di-n-octadecyl urea.

4. A lubricating grease as described in claim 1 wherein the minor amount of a thickening agent is a minor amount of  $\text{CaCO}_3$ .

of  $\text{SiO}_2$ .

**References Cited in the file of this patent**

UNITED STATES PATENTS

- |              |                |       |                |
|--------------|----------------|-------|----------------|
| 1,437,027    | Tanberg        | ----- | Nov. 28, 1922  |
| 2,050,582    | Orthner et al. | ----- | Aug. 11, 1936  |
| 2,195,167    | Egerton        | ----- | Mar. 26, 1940  |
| 2,257,717    | Olin           | ----- | Sept. 30, 1941 |
| 50 2,276,696 | Olin           | ----- | Mar. 17, 1942  |
| 2,668,758    | Roos           | ----- | Feb. 9, 1954   |
| 2,710,841    | Swakon et al.  | ----- | June 14, 1955  |

## FOREIGN PATENTS

- 55 17,501 Great Britain ----- Feb. 11, 1915  
802,941 Great Britain ----- Oct. 15, 1958